

Nov. 18, 1924.

1,515,949

C. P. HEGAN

AIR CLEANING MATERIAL AND PROCESS OF MAKING THE SAME

Filed March 27, 1924



Inventor:

1884 Chester P. Hagan,  
Byron Townsend & Brickerstein,

Attorneys.

## UNITED STATES PATENT OFFICE.

CHESTER P. HEGAN, OF LOUISVILLE, KENTUCKY, ASSIGNOR TO REED AIR FILTER COMPANY, OF LOUISVILLE, KENTUCKY, A CORPORATION OF KENTUCKY.

## AIR-CLEANING MATERIAL AND PROCESS OF MAKING THE SAME.

Application filed March 27, 1924. Serial No. 702,405.

*To all whom it may concern:*

Be it known that I, CHESTER P. HEGAN, a citizen of the United States, residing at 1267 First Street, Louisville, in the county of Jefferson and State of Kentucky, have invented certain new and useful Improvements in Air-Cleaning Materials and Processes of Making the Same, of which the following is a specification.

10 The invention relates to air cleaning material of the same general type as that described in the patent to Reed, No. 1,483,379, Feb. 12, 1924.

An object of the invention is to provide 15 a fibrous mass of air cleaning material, the individual metal fibers of which are protected by and bonded together by a metallic film. A further object of the invention is to provide a metal coated fibrous mass in 20 which the percentage of voids progressively decreases from one face to the opposite face of the mass. The invention also contemplates a novel method of forming a filtering mass having the characteristics specified 25 above.

It is well recognized that fibrous material such as steel wool is a very efficient 30 medium for the cleansing of air and gas, particularly when the fibrous material is coated with oil or other viscous fluids. Filters formed of metal fibers are open to the objection however that the individual fibers may shift position or mat down with a resultant increase in the air resistance.

35 As the individual fibers are fragile, they break up while in use, and such breakage may result in the formation of cracks extending through the mass, especially after the fibers have become more or less closely 40 matted. It is obvious that such matting or cracking of the filter mass renders the filter inefficient or inoperative and that the mass must be discarded since it cannot be restored to its original efficiency by the usual 45 cleaning processes.

To overcome these difficulties, I bond the individual fibers to each other by coating the fibers with a metal or alloy, which is preferably acid and corrosion resistant. 50 The metal coating upon the fibers bonds the mass into an integral structure which will

retain its shape and arrangement under the severest conditions of use, such for example as are encountered when the filter is located at the intake of an air compressor. The individual fibers are reinforced by the metal coating and will not be broken by the repeated pulsations set up by the compressor. 55

The fibrous mass is preferably assembled in a filter cell or unit before the coating operation and the entire cell is immersed in pickling baths of the usual type, then in a flux such as zinc chloride solution and finally in a bath of molten metal or alloy, for example, an alloy of lead, 94%, and antimony, 6%. Upon removal from the molten bath, the excess coating material may be removed in various ways, such as by shaking, by forcing the cell into a bath of heated oil or by blowing superheated air through 70 the cell.

For a better understanding of the novel air cleaning material and the process of producing the same, attention is called to the accompanying drawing, in which 75

Fig. 1 is a sectional view of a filter cell containing fibrous material embodying my invention;

Fig. 2 is a diagrammatic view of apparatus which may be employed in forming 80 the filtering material.

In the drawings, the numeral 1 designates the open frame of a filter unit or cell within which is arranged a mass of fibrous material 2. Wire screens 3, or other foraminous sheets are provided at the inlet and outlet faces of the frame to support the fibrous material before and during the coating operation, and these foraminous sheets also act as reinforcements in the finished 90 cell. 85

Although the metal coating may be applied to the fibrous material before it is assembled in a filter unit, I prefer to complete the mechanical assembly of the unit 95 before coating the metal wool. Apparatus for coating the assembled units is shown diagrammatically in Fig. 2, and comprises a flux tank 4, a tank 5 for holding the molten metal or alloy, a grating 6 resting 100 upon a frame 7 which is oscillated vertically by cams 8, and a tank 9 for holding hot

water into which the coated cell is discharged for cleaning and cooling. The shaking mechanism is located within a hood or oven 10 through which pass the products of combustion from the heaters arranged beneath the several tanks, and the oven is provided with a damper 11 for regulating the oven temperature. The inlet door 12 and outlet door 13 of the oven swing shut 10 by gravity and may be opened by the pressure or impact of a cell against the doors. The filter cells may be conveyed to the coating apparatus from the pickling vats, not shown, by an overhead traveler 14, which 15 traveler is also used for handling the filters during the coating process. After immersion in the flux tanks, the cells are transferred to the metal tank, and after a short immersion are then transferred to an inclined chute 15 from which they slide into the oven. The chute 15 preferably consists of spaced members, as angle bars, which engage only the opposite edges of the filter 20 in order that excess molten metal may drain from the filter onto the chute 16, which returns the metal to the tank 5. The shaking of the filter upon the rapping table facilitates the draining off of the excess metal which clings to the surface of the 25 metal fibers when the filter is removed from the molten bath. The excess metal drains from the filter, passing through the grating 6 into a pan 17. After a sufficient time, the loose grating 6 is tipped by any convenient 30 means to an angle sufficient to cause the filter to slide by gravity against the outlet door 13, which opens under the impact and allows the filter to slide into the tank 9 for cooling and rinsing. The removal and drying 35 of the filter complete the process.

Due to the use of products of combustion for heating the oven, the freshly deposited coating does not oxidize but remains as a bright, impervious metallic film upon the 40 individual fibers. The fibers are protected against corrosion and are bonded together so firmly that they will not shift position, mat or break under hard usage. A further and exceedingly desirable result is obtained 45 when metal fiber is treated by this process, i. e.; the fibers are more dense at one side of the filter than at the other. By lifting the cell from the molten bath in a horizontal position and with the inlet face of the cell 50 up, the excess metal in draining from the cell packs the fibers tighter at the outlet face of the cell. The progressive decrease in the 55 percentage of voids which is thus secured results in a more even distribution of the collected solids throughout the filter and allows the collection of the maximum amount of material with the lowest resistance to air or flow.

The same results may be obtained when

the excess metal is removed by passing 65 superheated air through the cell from the inlet face, the cell being arranged horizontally and with the inlet face up or by forcing the cell into a bath of heated oil. It will be apparent that the variation in 70 density which is secured by the novel process of treating a mass of metal fibers of substantially uniform density may be controlled by regulation of the temperature in the oven or the rate at which the excess metal is 75 drained or forced from the metal fibers.

While I have specified a particular lead-antimony alloy as a preferred coating material, it will be understood that these metals may be alloyed in varying proportions or 80 that other metals or alloys may be employed. Any one of the metals or alloys which may serve to bond the metal fibers together and render them less frangible is to be considered as a coating "metal", as such term 85 is employed in the following claims.

I claim:

1. A filter mass comprising metal fiber, the fibers of which are bonded together by a metallic coating which covers the individual fibers.

2. A filter mass comprising metal fiber, the individual fibers of which are covered with and bonded together by a coating of a different metal.

3. A filter mass as claimed in claim 2 in which the coating metal comprises a lead-antimony alloy.

4. A filter mass comprising metal fiber, the density of said mass progressively varying from one face to the other face of said mass, and means for maintaining the varying density of said mass.

5. A filter mass as claimed in claim 4, wherein said means comprises a film of 105 metal coating the individual fibers of said mass.

6. A filter cell comprising an open frame, foraminous sheets covering the faces of the frame, and a body of metal fibers filling 110 said frame, the individual fibers being coated with and bonded together by a different metal.

7. A filter cell as claimed in claim 6 wherein said body of coated metal fibers 115 progressively increases in density from the inlet towards the outlet face of the cell.

8. A filter cell as claimed in claim 6 wherein said metal fibers comprise steel wool and said coating metal comprises a 120 lead-antimony alloy.

9. A filter cell comprising an open frame, foraminous sheets covering the faces of said frame, and a body of metal fiber filling said frame, said metal fiber being of progressively increasing density from the inlet towards the outlet face of said cell and the individual fibers of said metal fiber being

coated with and bonded together by a lead-antimony alloy.

10. The process of producing filter material of progressively varying density from a body of metal fiber of substantially uniform density, which comprises dipping the metal fiber in a bath of metal, and displacing the excess metal from the face at which the least density is desired towards and out of the body of metal fiber at the face at which the greatest density is desired. In testimony whereof, I affix my signature.

CHESTER P. HEGAN.